

April 5, 1938.

J. M. OLIN ET AL

2,113,280

PROCESS FOR MANUFACTURING SHOT

Filed May 23, 1933



INVENTOR

John M. Olin

Philip A. Smith

BY

Pennie, Davis, Marvin & Edmunds

ATTORNEYS

## UNITED STATES PATENT OFFICE

2,113,280

## PROCESS FOR MANUFACTURING SHOT

John M. Olin, Alton, Ill., and Philip A. Smith, Hamden, Conn., assignors to Winchester Repeating Arms Company, New Haven, Conn., a corporation of Maryland

Application May 23, 1933, Serial No. 672,395

4 Claims. (Cl. 83—91)

This invention relates to shot and more particularly to shot formed of zinc or zinc alloys. Heretofore there has been no known method of producing commercial zinc shot of the sizes ordinarily used in shot gun cartridges. In our co-pending application Serial No. 672,394 filed May 23, 1933 we have disclosed and claimed a process of making shot wherein the globules or particles of molten metal enter the top of the shot tower in an atmosphere of inert gases. While our co-pending application is directed to the use of this process in connection with any desired metal and specifically to the use of the process in connection with scrap lead, it may also be employed in the manufacture of zinc shot and by this process we are able to obtain commercial production of zinc shot of desired sizes and the percentage of pellets discarded because of irregular shape is not substantially higher than the percentage discarded in the present practice of making lead shot.

In carrying out our invention we employ apparatus substantially similar to that now used in the manufacture of lead shot wherein a perforated drip pan is provided at the top of the shot tower and the molten metal is fed into the drip pan and allowed to pass into the top of the tower through the openings in the pan. In the usual practice of making lead shot wherein commercially pure lead is employed in combination with certain amounts of arsenic, the globules or particles of lead which pass through the openings in the drip pan fall through a column of air in the tower and during this fall they assume a spherical shape. As stated above, if the shot tower is filled with air and the present commonly used process is applied to zinc, the particles do not assume a spherical shape but are tear-shaped or have small tails or whiskers. We have found that spherical pellets of zinc may be obtained by maintaining a reducing or inert atmosphere in the tower, or at least in the upper portion of the tower where the particles or globules first assume a spherical shape. Any suitable reducing or inert gas may be employed for this purpose. As examples of reducing gases we may employ illuminating gas, water gas, producer gas, butane, hydrogen or any equivalents of these materials. As an inert medium through which the particles of zinc may pass we may employ nitrogen. Where a reducing gas is employed it is necessary to take precaution not to develop an explosive mixture in the shot tower.

In the accompanying drawing we have illustrated a shot gun cartridge forming a part of

this invention and have also illustrated apparatus for carrying out the process of producing zinc shot. In the drawing:

The figure is a diagrammatic view, in section, of the upper portion of a shot tower provided with means for maintaining the desired conditions in the shot tower.

As stated, the process described in our co-pending application, Serial No. 672,394 may be employed in the manufacture of the zinc shot and the application of such process to the manufacture of such shot is claimed herein. Referring to the drawing the apparatus disclosed therein consists of the upper portion of a conventional shot tower with means for supplying the inert or reducing gas to the tower. The floor 10 at the top of the tower is provided with an opening into which a skeleton frame 11 loosely fits. This frame forms a support for the drip pan or colander 12 and also supports the upper end of cylinder 13. An inlet pipe 14 opens into the cylinder near the top and is connected to a source of inert or reducing gas. In practicing the process the gas is supplied in sufficient amount to fill the cylinder 13 and maintain the desired non-oxidizing atmosphere at the perforations in the drip pan. The cylinder 13 is of the usual construction and its length is ordinarily dependent on the size of the holes in the drip pan and the average size of the pellets desired in that particular run of the shot tower. In carrying out the process, zinc or a zinc alloy is fed to the drip pan in molten condition, preferably syphoned from a large fusion kettle (not shown), through a feed pipe 15 in accordance with the usual practice. The metal drips through the perforations in the bottom of the pan and immediately comes in contact with the atmosphere of reducing gas or inert gas. Under such conditions we have found that the globules or particles of zinc coming from the bottom of the drip pan will assume a spherical form. During the operation of the tower it is advantageous to prevent the danger of explosion by burning the gas at the bottom of the cylinder as indicated at 16. The pellets or shot formed descend through the cylinder and the globules congeal sufficiently to prevent deformation when they strike the water at the bottom of the tower. The pellets fall into a water bath 20 as is the usual practice in the manufacture of shot and are cooled. They are removed from the water tank, dried and sorted to remove imperfectly shaped pellets in the usual manner.

While we are unable to offer a sound scientific explanation of the reason why spherical pellets

of zinc may be obtained when a reducing gas or an inert gas is maintained in the cylinder instead of air, we believe that the true explanation centers around certain obscure principles of the laws of surface tension as applied to a molten metal body falling freely. Whatever may be the true explanation of these principles there is the net commercial result that we are able to form zinc pellets in substantially the same manner that has heretofore been employed in the manufacture of lead shot. As stated above, this permits us to employ zinc shot either alone or in admixture with lead shot or other metal shot in the manufacture of shot gun cartridges and to obtain ballistic characteristics for cartridges of various calibers that have heretofore been impossible.

The zinc shot so obtained is spherical in shape according to the usual shot making practice and the percentage of pellets discarded because of irregular shape is not substantially higher than the percentage discarded in the present practice of making lead shot. Scrap zinc may be employed in the process and the cost of raw material may be, therefore, reduced considerably below those now prevailing in ordinary shot making.

While we have disclosed the invention in connection with the conventional type of shot gun cartridge employing a paper tube, it will, of course, be apparent that the invention can be employed in connection with shot shells of the type now made in which a brass cartridge case is employed in place of the paper type.

35 We claim:

1. The process of making substantially spherical shot suitable for use in the manufacture of shot gun cartridges which comprises separating

molten zinc into globules at the top of a shot tower, and protecting said zinc globules from contact with oxygen during at least the initial part of their flight down said shot tower, whereby said globules are caused to assume a substantially spherical shape during the initial part of their flight. 5

2. The process of making substantially spherical shot suitable for use in the manufacture of shot gun cartridges which comprises separating 10 molten zinc into globules at the top of a shot tower and maintaining an atmosphere of reducing gas in a portion of the tower through which the fused zinc globules start their flight, whereby said globules are caused to assume a 15 substantially spherical shape during the initial part of their flight.

3. The process of making substantially spherical shot suitable for use in the manufacture of shot gun cartridges which comprises introducing 20 molten zinc into a perforated drip pan at the top of a shot tower, permitting the molten zinc to flow through the perforations into the top of the shot tower, and protecting said molten zinc from contact with oxygen during at 25 least the initial part of its flight down said shot tower, whereby said globules are caused to assume a substantially spherical shape during the initial part of their flight.

4. In the process of making substantially 30 spherical shot for use in the manufacture of shot gun cartridges from zinc, the step which comprises protecting the zinc globules from contact with oxygen during at least the initial portion of their flight down a shot tower. 35

JOHN M. OLIN.  
PHILIP A. SMITH.